

# United States Patent Office

3,068,099

Patented Dec. 11, 1962

1

3,068,099

## PHOTOGRAPHIC SILVER HALIDE EMULSIONS CONTAINING THIOETHERS OF SATURATED OXYGEN HETEROCYCLES AS STABILIZERS AND ANTIFOGGANTS

Guenther H. Klinger, Binghamton, N.Y., assignor to  
General Aniline & Film Corporation, New York, N.Y.,  
a corporation of Delaware

No Drawing. Filed Feb. 1, 1961, Ser. No. 36,280

6 Claims. (Cl. 96—63)

This invention relates to light sensitive silver halide photographic emulsions which contain as stabilizers and antifogants thioethers of fully saturated oxygen-containing heterocyclic ring systems having one nuclear oxygen atom and 4 to 5 carbon atoms in the ring. The invention also relates to methods of preparing such photographic emulsions and to photographic elements prepared therefrom.

It is known that silver halide photographic emulsions, when stored for any length of time, become spontaneously developable without exposure to light. The degree of developability depends on the storage conditions. When photographic elements containing such excessively aged emulsions are exposed and developed, there is produced, even in the unexposed areas of the plate, a certain quantity of developed silver. Optical opacity produced in this manner is commonly referred to as fog, and emulsions which gave rise to this condition are designated as fogged emulsions.

This photographic phenomenon has long engaged the attention of skilled artisans in the field, and numerous reasons and theories have been enunciated to account for this peculiarity of photographic emulsions. For instance, it is generally known that conditions of excessive humidity during storage aggravate or accelerate the formation of fog. In fact, it is a common practice to actually test photographic emulsions by exposing them to excessive humidity and temperature in order to ascertain their tendency toward fog formation. Such information is, of course, very important since emulsions may be subjected to the aforescribed conditions when used and stored in tropical climes. Photographic fog can also be produced by exposure to chemicals such as hydrogen, sulfide or other reactive sulfur gaseous compounds, including strongly reducing materials. Many of these materials are found in the atmosphere.

A large number of substances have been proposed as being effective in retarding or preventing fog when such entities are incorporated in light sensitive silver halide emulsions. These photographic adjuncts are commonly referred to as antifogants or stabilizers, and are often compounds which have a mercapto function as the reactive group in their molecular structure. Although mercapto compounds may be effective in reducing or preventing fog, they almost always depress development rate in the exposed areas resulting in diminished speed. To overcome this dilemma, it has been suggested to employ a dual development technique based on the difference of developability of exposed versus fogged emulsion.

It is well known that during photographic development, fog generally develops at a lower rate than that of the usable density. This differential developability can be utilized by initially developing the photographic material in a developer which contains no stabilizers and as soon as fog development begins further development can be continued in a developer free of mercapto stabilizers. In this way, it is possible to gain higher usable density while maintaining a lower fog level. However, the use of two separate developing operations is impractical and tedious. A modification of the two stage developer technique locates non-diffusing mercapto stabilizers in a gel-

2

tin undercoat. In this system, the stabilizers will slowly migrate into the silver halide layer during normal development. The object is to adjust diffusion time to such a rate that stabilizers become available or diffuse into

5 the emulsion layer at about the time that the main development is consummated so that the stabilizers will arrive on the scene to retard fog development which as previously pointed out lags behind normal development. Although this system is sound in principle, it is difficult to  
10 reduce to practice, mainly because all known mercapto stabilizers diffuse very rapidly, even during the coating operations, and, consequently depress normal photographic development with concomitant reduction in usable density.

15 I have now discovered a way of utilizing the stabilizing action and fog inhibiting properties of mercapto compounds while at the same time eliminating the deleterious photographic side effects normally associated with these adjuncts, i.e., developer suppression in the exposed areas  
20 of a silver halide emulsion with concomitant reduction in photographic speed.

The use of these mercapto compounds to inhibit fog and to stabilize photographic emulsions while simultaneously maintaining the speed and sensitivity of said emulsion  
25 constitutes the objects and purposes of this invention.

Other objects and purposes will become apparent as the description proceeds.

I have now discovered that mercapto compounds, when employed in the form of their thioethers, particularly  
30 their tetrahydropyranthioethers, are excellent antifogants and stabilizers for silver halide emulsions without the usual effect of diminishing photographic speed by retarding development in the exposed areas. Moreover, these mercapto ethers are effective in retarding speed loss during the aging of emulsions and are thus effective stabilizers as well as antifogants.

Exemplary tetrahydropyranthioethers, the use of which is contemplated herein can be represented by the following formula:



45 wherein R represents an alkyl group of from 1 to 20 carbon atoms such as methyl, ethyl, propyl, butyl, amyl, hexyl, heptyl, nonyl, decyl, lauryl, tetradecyl, cetyl, octadecyl, etc., an aralkyl group such as benzyl, phenethyl, etc., a cycloalkyl group such as cyclopentyl, cyclohexyl, etc., an aryl group such as a monocyclic or bicyclic aromatic hydrocarbon radical, etc., a heterocyclic ring system of the thiothiazole series, e.g., thiazole, 4-methylthiazole, 4-phenylthiazole, 5-methylthiazole, 5-phenylthiazole, 4,5-dimethylthiazole, 4,5-diphenylthiazole, 4-(2-chlorophenyl)thiazole, etc., those of the benzothiazole series, e.g., benzothiazole, 4-chlorobenzothiazole, 5-chlorobenzothiazole, 6-chlorobenzothiazole, 4-methylbenzothiazole, 5-methylbenzothiazole, 5-bromobenzothiazole, 4-phenylbenzothiazole, 5-phenylbenzothiazole, 5-methoxybenzothiazole, 6-methoxybenzothiazole, 4-ethoxybenzothiazole, tetrahydrobenzothiazole, 6-hydroxybenzothiazole, etc., those of the naphthothiazole series, e.g.,  $\beta$ -naphthothiazole,  $\alpha$ -naphthothiazole, 5-methoxy- $\beta$ -naphthothiazole, 5-ethoxy- $\beta$ -naphthothiazole, 8-methoxy- $\alpha$ -naphthothiazole, etc.,  
50 those of the benzoxazole series, e.g., benzoxazole 5-chlorobenzoxazole, 5-methylbenzoxazole, 5-phenylbenzoxazole, 6-methylbenzoxazole, 4,5-dimethylbenzoxazole, 5-chlorobenzoxazole, 6-methoxybenzoxazole, 6-hydroxybenzoxazole, etc., those of the benzoselenazole series, e.g., benzoselenazole, 5-chlorobenzoselenazole, 5-methoxybenzose-  
55 lenazole, etc., those of the quinoline series, e.g., quinoline,  
60 those of the isoquinoline series, e.g., isoquinoline, 5-methoxyisoquinoline, 5-ethoxyisoquinoline, 8-methoxyisoquinoline, etc., those of the carbazole series, e.g., carbazole, 5-methoxycarbazole, 5-ethoxy-  
65 carbazole, 8-methoxy- $\alpha$ -carbazole, etc., those of the indole series, e.g., indole, 5-methoxyindole, 5-ethoxyindole, 8-methoxyindole, etc., those of the carbazoles, e.g., carbazole, 5-methoxycarbazole, 5-ethoxy-  
70 carbazole, 8-methoxy- $\alpha$ -carbazole, etc., those of the indoles, e.g., indole, 5-methoxyindole, 5-ethoxyindole, 8-methoxyindole, etc., those of the indolizine series, e.g., indolizine, 5-methoxyindolizine, 5-ethoxy-  
75 indolizine, 8-methoxyindolizine, etc., those of the purine series, e.g., purine, 6-methoxypurine, 6-ethoxypurine, 8-methoxypurine, etc., those of the imidazole series, e.g., imidazole, 5-methoxyimidazole, 5-ethoxy-  
80 imidazole, 8-methoxyimidazole, etc., those of the imidazoles, e.g., imidazole, 5-methoxyimidazole, 5-ethoxy-  
85 imidazole, 8-methoxyimidazole, etc., those of the imidazoles, e.g., imidazole, 5-methoxyimidazole, 5-ethoxy-  
90 imidazole, 8-methoxyimidazole, etc., those of the imidazoles, e.g., imidazole, 5-methoxyimidazole, 5-ethoxy-  
95 imidazole, 8-methoxyimidazole, etc., those of the imidazoles, e.g., imidazole, 5-methoxyimidazole, 5-ethoxy-  
100 imidazole, 8-methoxyimidazole, etc., those of the imidazoles, e.g., imidazole, 5-methoxyimidazole, 5-ethoxy-  
105 imidazole, 8-methoxyimidazole, etc., those of the imidazoles, e.g., imidazole, 5-methoxyimidazole, 5-ethoxy-  
110 imidazole, 8-methoxyimidazole, etc., those of the imidazoles, e.g., imidazole, 5-methoxyimidazole, 5-ethoxy-  
115 imidazole, 8-methoxyimidazole, etc., those of the imidazoles, e.g., imidazole, 5-methoxyimidazole, 5-ethoxy-  
120 imidazole, 8-methoxyimidazole, etc., those of the imidazoles, e.g., imidazole, 5-methoxyimidazole, 5-ethoxy-  
125 imidazole, 8-methoxyimidazole, etc., those of the imidazoles, e.g., imidazole, 5-methoxyimidazole, 5-ethoxy-  
130 imidazole, 8-methoxyimidazole, etc., those of the imidazoles, e.g., imidazole, 5-methoxyimidazole, 5-ethoxy-  
135 imidazole, 8-methoxyimidazole, etc., those of the imidazoles, e.g., imidazole, 5-methoxyimidazole, 5-ethoxy-  
140 imidazole, 8-methoxyimidazole, etc., those of the imidazoles, e.g., imidazole, 5-methoxyimidazole, 5-ethoxy-  
145 imidazole, 8-methoxyimidazole, etc., those of the imidazoles, e.g., imidazole, 5-methoxyimidazole, 5-ethoxy-  
150 imidazole, 8-methoxyimidazole, etc., those of the imidazoles, e.g., imidazole, 5-methoxyimidazole, 5-ethoxy-  
155 imidazole, 8-methoxyimidazole, etc., those of the imidazoles, e.g., imidazole, 5-methoxyimidazole, 5-ethoxy-  
160 imidazole, 8-methoxyimidazole, etc., those of the imidazoles, e.g., imidazole, 5-methoxyimidazole, 5-ethoxy-  
165 imidazole, 8-methoxyimidazole, etc., those of the imidazoles, e.g., imidazole, 5-methoxyimidazole, 5-ethoxy-  
170 imidazole, 8-methoxyimidazole, etc., those of the imidazoles, e.g., imidazole, 5-methoxyimidazole, 5-ethoxy-  
175 imidazole, 8-methoxyimidazole, etc., those of the imidazoles, e.g., imidazole, 5-methoxyimidazole, 5-ethoxy-  
180 imidazole, 8-methoxyimidazole, etc., those of the imidazoles, e.g., imidazole, 5-methoxyimidazole, 5-ethoxy-  
185 imidazole, 8-methoxyimidazole, etc., those of the imidazoles, e.g., imidazole, 5-methoxyimidazole, 5-ethoxy-  
190 imidazole, 8-methoxyimidazole, etc., those of the imidazoles, e.g., imidazole, 5-methoxyimidazole, 5-ethoxy-  
195 imidazole, 8-methoxyimidazole, etc., those of the imidazoles, e.g., imidazole, 5-methoxyimidazole, 5-ethoxy-  
200 imidazole, 8-methoxyimidazole, etc., those of the imidazoles, e.g., imidazole, 5-methoxyimidazole, 5-ethoxy-  
205 imidazole, 8-methoxyimidazole, etc., those of the imidazoles, e.g., imidazole, 5-methoxyimidazole, 5-ethoxy-  
210 imidazole, 8-methoxyimidazole, etc., those of the imidazoles, e.g., imidazole, 5-methoxyimidazole, 5-ethoxy-  
215 imidazole, 8-methoxyimidazole, etc., those of the imidazoles, e.g., imidazole, 5-methoxyimidazole, 5-ethoxy-  
220 imidazole, 8-methoxyimidazole, etc., those of the imidazoles, e.g., imidazole, 5-methoxyimidazole, 5-ethoxy-  
225 imidazole, 8-methoxyimidazole, etc., those of the imidazoles, e.g., imidazole, 5-methoxyimidazole, 5-ethoxy-  
230 imidazole, 8-methoxyimidazole, etc., those of the imidazoles, e.g., imidazole, 5-methoxyimidazole, 5-ethoxy-  
235 imidazole, 8-methoxyimidazole, etc., those of the imidazoles, e.g., imidazole, 5-methoxyimidazole, 5-ethoxy-  
240 imidazole, 8-methoxyimidazole, etc., those of the imidazoles, e.g., imidazole, 5-methoxyimidazole, 5-ethoxy-  
245 imidazole, 8-methoxyimidazole, etc., those of the imidazoles, e.g., imidazole, 5-methoxyimidazole, 5-ethoxy-  
250 imidazole, 8-methoxyimidazole, etc., those of the imidazoles, e.g., imidazole, 5-methoxyimidazole, 5-ethoxy-  
255 imidazole, 8-methoxyimidazole, etc., those of the imidazoles, e.g., imidazole, 5-methoxyimidazole, 5-ethoxy-  
260 imidazole, 8-methoxyimidazole, etc., those of the imidazoles, e.g., imidazole, 5-methoxyimidazole, 5-ethoxy-  
265 imidazole, 8-methoxyimidazole, etc., those of the imidazoles, e.g., imidazole, 5-methoxyimidazole, 5-ethoxy-  
270 imidazole, 8-methoxyimidazole, etc., those of the imidazoles, e.g., imidazole, 5-methoxyimidazole, 5-ethoxy-  
275 imidazole, 8-methoxyimidazole, etc., those of the imidazoles, e.g., imidazole, 5-methoxyimidazole, 5-ethoxy-  
280 imidazole, 8-methoxyimidazole, etc., those of the imidazoles, e.g., imidazole, 5-methoxyimidazole, 5-ethoxy-  
285 imidazole, 8-methoxyimidazole, etc., those of the imidazoles, e.g., imidazole, 5-methoxyimidazole, 5-ethoxy-  
290 imidazole, 8-methoxyimidazole, etc., those of the imidazoles, e.g., imidazole, 5-methoxyimidazole, 5-ethoxy-  
295 imidazole, 8-methoxyimidazole, etc., those of the imidazoles, e.g., imidazole, 5-methoxyimidazole, 5-ethoxy-  
300 imidazole, 8-methoxyimidazole, etc., those of the imidazoles, e.g., imidazole, 5-methoxyimidazole, 5-ethoxy-  
305 imidazole, 8-methoxyimidazole, etc., those of the imidazoles, e.g., imidazole, 5-methoxyimidazole, 5-ethoxy-  
310 imidazole, 8-methoxyimidazole, etc., those of the imidazoles, e.g., imidazole, 5-methoxyimidazole, 5-ethoxy-  
315 imidazole, 8-methoxyimidazole, etc., those of the imidazoles, e.g., imidazole, 5-methoxyimidazole, 5-ethoxy-  
320 imidazole, 8-methoxyimidazole, etc., those of the imidazoles, e.g., imidazole, 5-methoxyimidazole, 5-ethoxy-  
325 imidazole, 8-methoxyimidazole, etc., those of the imidazoles, e.g., imidazole, 5-methoxyimidazole, 5-ethoxy-  
330 imidazole, 8-methoxyimidazole, etc., those of the imidazoles, e.g., imidazole, 5-methoxyimidazole, 5-ethoxy-  
335 imidazole, 8-methoxyimidazole, etc., those of the imidazoles, e.g., imidazole, 5-methoxyimidazole, 5-ethoxy-  
340 imidazole, 8-methoxyimidazole, etc., those of the imidazoles, e.g., imidazole, 5-methoxyimidazole, 5-ethoxy-  
345 imidazole, 8-methoxyimidazole, etc., those of the imidazoles, e.g., imidazole, 5-methoxyimidazole, 5-ethoxy-  
350 imidazole, 8-methoxyimidazole, etc., those of the imidazoles, e.g., imidazole, 5-methoxyimidazole, 5-ethoxy-  
355 imidazole, 8-methoxyimidazole, etc., those of the imidazoles, e.g., imidazole, 5-methoxyimidazole, 5-ethoxy-  
360 imidazole, 8-methoxyimidazole, etc., those of the imidazoles, e.g., imidazole, 5-methoxyimidazole, 5-ethoxy-  
365 imidazole, 8-methoxyimidazole, etc., those of the imidazoles, e.g., imidazole, 5-methoxyimidazole, 5-ethoxy-  
370 imidazole, 8-methoxyimidazole, etc., those of the imidazoles, e.g., imidazole, 5-methoxyimidazole, 5-ethoxy-  
375 imidazole, 8-methoxyimidazole, etc., those of the imidazoles, e.g., imidazole, 5-methoxyimidazole, 5-ethoxy-  
380 imidazole, 8-methoxyimidazole, etc., those of the imidazoles, e.g., imidazole, 5-methoxyimidazole, 5-ethoxy-  
385 imidazole, 8-methoxyimidazole, etc., those of the imidazoles, e.g., imidazole, 5-methoxyimidazole, 5-ethoxy-  
390 imidazole, 8-methoxyimidazole, etc., those of the imidazoles, e.g., imidazole, 5-methoxyimidazole, 5-ethoxy-  
395 imidazole, 8-methoxyimidazole, etc., those of the imidazoles, e.g., imidazole, 5-methoxyimidazole, 5-ethoxy-  
400 imidazole, 8-methoxyimidazole, etc., those of the imidazoles, e.g., imidazole, 5-methoxyimidazole, 5-ethoxy-  
405 imidazole, 8-methoxyimidazole, etc., those of the imidazoles, e.g., imidazole, 5-methoxyimidazole, 5-ethoxy-  
410 imidazole, 8-methoxyimidazole, etc., those of the imidazoles, e.g., imidazole, 5-methoxyimidazole, 5-ethoxy-  
415 imidazole, 8-methoxyimidazole, etc., those of the imidazoles, e.g., imidazole, 5-methoxyimidazole, 5-ethoxy-  
420 imidazole, 8-methoxyimidazole, etc., those of the imidazoles, e.g., imidazole, 5-methoxyimidazole, 5-ethoxy-  
425 imidazole, 8-methoxyimidazole, etc., those of the imidazoles, e.g., imidazole, 5-methoxyimidazole, 5-ethoxy-  
430 imidazole, 8-methoxyimidazole, etc., those of the imidazoles, e.g., imidazole, 5-methoxyimidazole, 5-ethoxy-  
435 imidazole, 8-methoxyimidazole, etc., those of the imidazoles, e.g., imidazole, 5-methoxyimidazole, 5-ethoxy-  
440 imidazole, 8-methoxyimidazole, etc., those of the imidazoles, e.g., imidazole, 5-methoxyimidazole, 5-ethoxy-  
445 imidazole, 8-methoxyimidazole, etc., those of the imidazoles, e.g., imidazole, 5-methoxyimidazole, 5-ethoxy-  
450 imidazole, 8-methoxyimidazole, etc., those of the imidazoles, e.g., imidazole, 5-methoxyimidazole, 5-ethoxy-  
455 imidazole, 8-methoxyimidazole, etc., those of the imidazoles, e.g., imidazole, 5-methoxyimidazole, 5-ethoxy-  
460 imidazole, 8-methoxyimidazole, etc., those of the imidazoles, e.g., imidazole, 5-methoxyimidazole, 5-ethoxy-  
465 imidazole, 8-methoxyimidazole, etc., those of the imidazoles, e.g., imidazole, 5-methoxyimidazole, 5-ethoxy-  
470 imidazole, 8-methoxyimidazole, etc., those of the imidazoles, e.g., imidazole, 5-methoxyimidazole, 5-ethoxy-  
475 imidazole, 8-methoxyimidazole, etc., those of the imidazoles, e.g., imidazole, 5-methoxyimidazole, 5-ethoxy-  
480 imidazole, 8-methoxyimidazole, etc., those of the imidazoles, e.g., imidazole, 5-methoxyimidazole, 5-ethoxy-  
485 imidazole, 8-methoxyimidazole, etc., those of the imidazoles, e.g., imidazole, 5-methoxyimidazole, 5-ethoxy-  
490 imidazole, 8-methoxyimidazole, etc., those of the imidazoles, e.g., imidazole, 5-methoxyimidazole, 5-ethoxy-  
495 imidazole, 8-methoxyimidazole, etc., those of the imidazoles, e.g., imidazole, 5-methoxyimidazole, 5-ethoxy-  
500 imidazole, 8-methoxyimidazole, etc., those of the imidazoles, e.g., imidazole, 5-methoxyimidazole, 5-ethoxy-  
505 imidazole, 8-methoxyimidazole, etc., those of the imidazoles, e.g., imidazole, 5-methoxyimidazole, 5-ethoxy-  
510 imidazole, 8-methoxyimidazole, etc., those of the imidazoles, e.g., imidazole, 5-methoxyimidazole, 5-ethoxy-  
515 imidazole, 8-methoxyimidazole, etc., those of the imidazoles, e.g., imidazole, 5-methoxyimidazole, 5-ethoxy-  
520 imidazole, 8-methoxyimidazole, etc., those of the imidazoles, e.g., imidazole, 5-methoxyimidazole, 5-ethoxy-  
525 imidazole, 8-methoxyimidazole, etc., those of the imidazoles, e.g., imidazole, 5-methoxyimidazole, 5-ethoxy-  
530 imidazole, 8-methoxyimidazole, etc., those of the imidazoles, e.g., imidazole, 5-methoxyimidazole, 5-ethoxy-  
535 imidazole, 8-methoxyimidazole, etc., those of the imidazoles, e.g., imidazole, 5-methoxyimidazole, 5-ethoxy-  
540 imidazole, 8-methoxyimidazole, etc., those of the imidazoles, e.g., imidazole, 5-methoxyimidazole, 5-ethoxy-  
545 imidazole, 8-methoxyimidazole, etc., those of the imidazoles, e.g., imidazole, 5-methoxyimidazole, 5-ethoxy-  
550 imidazole, 8-methoxyimidazole, etc., those of the imidazoles, e.g., imidazole, 5-methoxyimidazole, 5-ethoxy-  
555 imidazole, 8-methoxyimidazole, etc., those of the imidazoles, e.g., imidazole, 5-methoxyimidazole, 5-ethoxy-  
560 imidazole, 8-methoxyimidazole, etc., those of the imidazoles, e.g., imidazole, 5-methoxyimidazole, 5-ethoxy-  
565 imidazole, 8-methoxyimidazole, etc., those of the imidazoles, e.g., imidazole, 5-methoxyimidazole, 5-ethoxy-  
570 imidazole, 8-methoxyimidazole, etc., those of the imidazoles, e.g., imidazole, 5-methoxyimidazole, 5-ethoxy-  
575 imidazole, 8-methoxyimidazole, etc., those of the imidazoles, e.g., imidazole, 5-methoxyimidazole, 5-ethoxy-  
580 imidazole, 8-methoxyimidazole, etc., those of the imidazoles, e.g., imidazole, 5-methoxyimidazole, 5-ethoxy-  
585 imidazole, 8-methoxyimidazole, etc., those of the imidazoles, e.g., imidazole, 5-methoxyimidazole, 5-ethoxy-  
590 imidazole, 8-methoxyimidazole, etc., those of the imidazoles, e.g., imidazole, 5-methoxyimidazole, 5-ethoxy-  
595 imidazole, 8-methoxyimidazole, etc., those of the imidazoles, e.g., imidazole, 5-methoxyimidazole, 5-ethoxy-  
600 imidazole, 8-methoxyimidazole, etc., those of the imidazoles, e.g., imidazole, 5-methoxyimidazole, 5-ethoxy-  
605 imidazole, 8-methoxyimidazole, etc., those of the imidazoles, e.g., imidazole, 5-methoxyimidazole, 5-ethoxy-  
610 imidazole, 8-methoxyimidazole, etc., those of the imidazoles, e.g., imidazole, 5-methoxyimidazole, 5-ethoxy-  
615 imidazole, 8-methoxyimidazole, etc., those of the imidazoles, e.g., imidazole, 5-methoxyimidazole, 5-ethoxy-  
620 imidazole, 8-methoxyimidazole, etc., those of the imidazoles, e.g., imidazole, 5-methoxyimidazole, 5-ethoxy-  
625 imidazole, 8-methoxyimidazole, etc., those of the imidazoles, e.g., imidazole, 5-methoxyimidazole, 5-ethoxy-  
630 imidazole, 8-methoxyimidazole, etc., those of the imidazoles, e.g., imidazole, 5-methoxyimidazole, 5-ethoxy-  
635 imidazole, 8-methoxyimidazole, etc., those of the imidazoles, e.g., imidazole, 5-methoxyimidazole, 5-ethoxy-  
640 imidazole, 8-methoxyimidazole, etc., those of the imidazoles, e.g., imidazole, 5-methoxyimidazole, 5-ethoxy-  
645 imidazole, 8-methoxyimidazole, etc., those of the imidazoles, e.g., imidazole, 5-methoxyimidazole, 5-ethoxy-  
650 imidazole, 8-methoxyimidazole, etc., those of the imidazoles, e.g., imidazole, 5-methoxyimidazole, 5-ethoxy-  
655 imidazole, 8-methoxyimidazole, etc., those of the imidazoles, e.g., imidazole, 5-methoxyimidazole, 5-ethoxy-  
660 imidazole, 8-methoxyimidazole, etc., those of the imidazoles, e.g., imidazole, 5-methoxyimidazole, 5-ethoxy-  
665 imidazole, 8-methoxyimidazole, etc., those of the imidazoles, e.g., imidazole, 5-methoxyimidazole, 5-ethoxy-  
670 imidazole, 8-methoxyimidazole, etc., those of the imidazoles, e.g., imidazole, 5-methoxyimidazole, 5-ethoxy-  
675 imidazole, 8-methoxyimidazole, etc., those of the imidazoles, e.g., imidazole, 5-methoxyimidazole, 5-ethoxy-  
680 imidazole, 8-methoxyimidazole, etc., those of the imidazoles, e.g., imidazole, 5-methoxyimidazole, 5-ethoxy-  
685 imidazole, 8-methoxyimidazole, etc., those of the imidazoles, e.g., imidazole, 5-methoxyimidazole, 5-ethoxy-  
690 imidazole, 8-methoxyimidazole, etc., those of the imidazoles, e.g., imidazole, 5-methoxyimidazole, 5-ethoxy-  
695 imidazole, 8-methoxyimidazole, etc., those of the imidazoles, e.g., imidazole, 5-methoxyimidazole, 5-ethoxy-  
700 imidazole, 8-methoxyimidazole, etc., those of the imidazoles, e.g., imidazole, 5-methoxyimidazole, 5-ethoxy-  
705 imidazole, 8-methoxyimidazole, etc., those of the imidazoles, e.g., imidazole, 5-methoxyimidazole, 5-ethoxy-  
710 imidazole, 8-methoxyimidazole, etc., those of the imidazoles, e.g., imidazole, 5-methoxyimidazole, 5-ethoxy-  
715 imidazole, 8-methoxyimidazole, etc., those of the imidazoles, e.g., imidazole, 5-methoxyimidazole, 5-ethoxy-  
720 imidazole, 8-methoxyimidazole, etc., those of the imidazoles, e.g., imidazole, 5-methoxyimidazole, 5-ethoxy-  
725 imidazole, 8-methoxyimidazole, etc., those of the imidazoles, e.g., imidazole, 5-methoxyimidazole, 5-ethoxy-  
730 imidazole, 8-methoxyimidazole, etc., those of the imidazoles, e.g., imidazole, 5-methoxyimidazole, 5-ethoxy-  
735 imidazole, 8-methoxyimidazole, etc., those of the imidazoles, e.g., imidazole, 5-methoxyimidazole, 5-ethoxy-  
740 imidazole, 8-methoxyimidazole, etc., those of the imidazoles, e.g., imidazole, 5-methoxyimidazole, 5-ethoxy-  
745 imidazole, 8-methoxyimidazole, etc., those of the imidazoles, e.g., imidazole, 5-methoxyimidazole, 5-ethoxy-  
750 imidazole, 8-methoxyimidazole, etc., those of the imidazoles, e.g., imidazole, 5-methoxyimidazole, 5-ethoxy-  
755 imidazole, 8-methoxyimidazole, etc., those of the imidazoles, e.g., imidazole, 5-methoxyimidazole, 5-ethoxy-  
760 imidazole, 8-methoxyimidazole, etc., those of the imidazoles, e.g., imidazole, 5-methoxyimidazole, 5-ethoxy-  
765 imidazole, 8-methoxyimidazole, etc., those of the imidazoles, e.g., imidazole, 5-methoxyimidazole, 5-ethoxy-  
770 imidazole, 8-methoxyimidazole, etc., those of the imidazoles, e.g., imidazole, 5-methoxyimidazole, 5-ethoxy-  
775 imidazole, 8-methoxyimidazole, etc., those of the imidazoles, e.g., imidazole, 5-methoxyimidazole, 5-ethoxy-  
780 imidazole, 8-methoxyimidazole, etc., those of the imidazoles, e.g., imidazole, 5-methoxyimidazole, 5-ethoxy-  
785 imidazole, 8-methoxyimidazole, etc., those of the imidazoles, e.g., imidazole, 5-methoxyimidazole, 5-ethoxy-  
790 imidazole, 8-methoxyimidazole, etc., those of the imidazoles, e.g., imidazole, 5-methoxyimidazole, 5-ethoxy-  
795 imidazole, 8-methoxyimidazole, etc., those of the imidazoles, e.g., imidazole, 5-methoxyimidazole, 5-ethoxy-  
800 imidazole, 8-methoxyimidazole, etc., those of the imidazoles, e.g., imidazole, 5-methoxyimidazole, 5-ethoxy-  
805 imidazole, 8-methoxyimidazole, etc., those of the imidazoles, e.g., imidazole, 5-methoxyimidazole, 5-ethoxy-  
810 imidazole, 8-methoxyimidazole, etc., those of the imidazoles, e.g., imidazole, 5-methoxyimidazole, 5-ethoxy-  
815 imidazole, 8-methoxyimidazole, etc., those of the imidazoles, e.g., imidazole, 5-methoxyimidazole, 5-ethoxy-  
820 imidazole, 8-methoxyimidazole, etc., those of the imidazoles, e.g., imidazole, 5-methoxyimidazole, 5-ethoxy-  
825 imidazole, 8-methoxyimidazole, etc., those of the imidazoles, e.g., imidazole, 5-methoxyimidazole, 5-ethoxy-  
830 imidazole, 8-methoxyimidazole, etc., those of the imidazoles, e.g., imidazole, 5-methoxyimidazole, 5-ethoxy-  
835 imidazole, 8-methoxyimidazole, etc., those of the imidazoles, e.g., imidazole, 5-methoxyimidazole, 5-ethoxy-  
840 imidazole, 8-methoxyimidazole, etc., those of the imidazoles, e.g., imidazole, 5-methoxyimidazole, 5-ethoxy-  
845 imidazole, 8-methoxyimidazole, etc., those of the imidazoles, e.g., imidazole, 5-methoxyimidazole, 5-ethoxy-  
850 imidazole, 8-methoxyimidazole, etc., those of the imidazoles, e.g., imidazole, 5-methoxyimidazole, 5-ethoxy-  
855 imidazole, 8-methoxyimidazole, etc., those of the imidazoles, e.g., imidazole, 5-methoxyimidazole, 5-ethoxy-  
860 imidazole, 8-methoxyimidazole, etc., those of the imidazoles, e.g., imidazole, 5-methoxyimidazole, 5-ethoxy-  
865 imidazole, 8-methoxyimidazole, etc., those of the imidazoles, e.g., imidazole, 5-methoxyimidazole, 5-ethoxy-  
870 imidazole, 8-methoxyimidazole, etc., those of the imidazoles, e.g., imidazole, 5-methoxyimidazole, 5-ethoxy-  
875 imidazole, 8-methoxyimidazole, etc., those of the imidazoles, e.g., imidazole, 5-methoxyimidazole, 5-ethoxy-  
880 imidazole, 8-methoxyimidazole, etc., those of the imidazoles, e.g., imidazole, 5-methoxyimidazole, 5-ethoxy-  
885 imidazole, 8-methoxyimidazole, etc., those of the imidazoles, e.g., imidazole, 5-methoxyimidazole, 5-ethoxy-  
890 imidazole, 8-methoxyimidazole, etc., those of the imidazoles, e.g., imidazole, 5-methoxyimidazole, 5-ethoxy-  
895 imidazole, 8-methoxyimidazole, etc., those of the imidazoles, e.g., imidazole, 5-methoxyimidazole, 5-ethoxy-  
900 imidazole, 8-methoxyimidazole, etc., those of the imidazoles, e.g., imidazole, 5-methoxyimidazole, 5-ethoxy-  
905 imidazole, 8-methoxyimidazole, etc., those of the imidazoles, e.g., imidazole, 5-methoxyimidazole, 5-ethoxy-  
910 imidazole, 8-methoxyimidazole, etc., those of the imidazoles, e.g., imidazole, 5-methoxyimidazole, 5-ethoxy-  
915 imidazole, 8-methoxyimidazole, etc., those of the imidazoles, e.g., imidazole, 5-methoxyimidazole, 5-ethoxy-  
920 imidazole, 8-methoxyimidazole, etc., those of the imidazoles, e.g., imidazole, 5-methoxyimidazole, 5-ethoxy-  
925 imidazole, 8-methoxyimidazole, etc., those of the imidazoles, e.g., imidazole, 5-methoxyimidazole, 5-ethoxy-  
930 imidazole, 8-methoxyimidazole, etc., those of the imidazoles, e.g., imidazole, 5-methoxyimidazole, 5-ethoxy-  
935 im



19.



20.



21.



22.



23.



The tetrahydropyran thioethers used in practicing the invention can be prepared by condensing the requisite 2-mercapto compound, e.g., a mercaptobenzothiazole with a dihydropyran in the presence of an acidic condensing agent such as p-toluenesulfonic acid. The reaction is conveniently carried out by refluxing the components in a suitable solvent after which the desired tetrahydropyran thioether is isolated by the well known methods of organic chemistry, such as crystallization or distillation.

An unusual characteristic of the tetrahydropyran thioethers contemplated herein is their cleavage in the presence of silver ion with regeneration of compounds containing free mercapto groups. It is this special property of tetrahydropyran thioethers which is considered to account for their efficiency as stabilizers and antifogants. However, any explanation in this connection is offered only as a theory and is not to be taken as limiting the invention to this particular mode of operation. It is possible that other mechanisms would provide a more complete interpretation of the behavior of the aforesaid entities.

Most photographic developers contain silver halide solvents, as for example sulfite. During the development process, small amounts of silver ions are in the solution due to the action of the aforementioned silver halide solvents. These silver ions are believed to split the tetrahydropyran ethers and to provide a molecule with a free mercapto group. At about the same time, chemical development of exposed grains begins to take place. There is no indication that the freshly generated free mercapto compound interferes with normal development as evidenced by an exceedingly low degree of fog density. Apparently the free mercapto compound is liberated at the optimum stage of development thus enabling it to exert maximum fog inhibiting power. It is not, however, formed or generated before normal development has proceeded to the optimum value. In other words, it is possible to harness the chemical reactions of development to regulate the production or generation of mercapto

compound, *in situ*, to procure optimum antifogging properties associated with such a compound while, at the same time, eliminating the usual speed loss caused by the presence of free mercapto additives. It will be appreciated that the theory or mechanism as above set forth is tentative and may not be correct in all its aspects, and may possibly be refined or elaborated subsequently. However, it is submitted the concept of freeing a mercapto compound so as to approximately coincide with the development action results in heretofore unobtainable advantages and the present invention thus represents a concept not previously contemplated by the prior art.

The aforementioned compounds can be utilized in various ways to secure beneficial effects and fog reduction. 15 For instance, the components can be incorporated in the silver halide emulsions as "ripening finals" or as "coating finals." "Ripening finals" are added during the ripening or the sensitivity increasing stage of the emulsion-making process. These additions may be made before, 20 during or after the double decomposition reaction between the soluble silver salt such as silver nitrate and the soluble halide such as potassium bromide. The latter reaction is, of course, carried out in the presence of a colloid carrier. By colloid carrier is intended the medium in 25 which is contained the light sensitive silver halide salts. Typical examples of these carriers include gelatin, PVA, solubilized casein, carboxymethyl cellulose, albumin and the like.

"Coating finals" are customarily added to the emulsion 30 just prior to coating on a suitable support such as glass, paper or film at a time when the emulsion is approaching its maximum sensitivity.

When incorporated directly in a silver halide emulsion, 35 the tetrahydropyran thioethers of the type described herein are preferably used in quantities ranging from 2 to 30 mg. per mole of silver bromide. It will, of course, be appreciated that the concentration will vary with various types of emulsion, and it may be desirable to determine the optimum concentration from case to case. 40 In some instances, it is advantageous to apply the antifogants and stabilizers in adjacent layers, e.g., in a separate undercoating layer or in the antiabrasion gelatin surface. Because of the physical separation between the silver halide emulsion layer and a separate undercoating layer, it is recommended that correspondingly larger quantities of antifogant be used when it is contained in undercoating surface. In some cases, it may be desirable to utilize the antifogants in one or all of the processing 45 baths or in various pre- and postbaths. Those skilled in the art will be in a position to ascertain the particular location of the antifogants for a given situation.

According to the invention, the antifogants and stabilizers can be advantageously employed in connection 50 with any type of photographic emulsion, e.g., non-sensitized, orthochromatic, panchromatic, X-ray emulsions, paper emulsions, color emulsions or the like. It has also been established that these compounds are usable in combination with other photographic adjuncts as exemplified by metal and noble sensitizers and in combination with a hydroxy polyphenoxy derivative of the type obtained 55 by reacting ethylene oxide with an alcohol phenol amine or the like, as described in U.S.P. 1,970,578.

The invention is illustrated by the following examples, but it is to be understood that the invention is not to be restricted thereto.

#### EXAMPLE I

A silver halide emulsion in gelatin containing 4% silver iodide and 96% silver bromide was prepared in a conventional manner and brought up to its maximum light sensitivity and then readied for coating. Finals were added, such as sensitizing dyes, hardening agents, or any various other photographic adjuncts commonly used in the art. The emulsion was divided into portions and to each was added varying quantities of the tetrahydropyran thioether of 2-mercaptopbenzothiazole and dihydro-

pyran. The emulsion samples contained about .4 mole of silver halide. The so-prepared samples were coated on a suitable cellulose ester base and dried. Samples of these film coatings were exposed in a Type IB sensitometer and developed in a developer of the following composition:

|                                 | Grams |
|---------------------------------|-------|
| Metol                           | 1.5   |
| Sodium sulfite (anhydrous)      | 45.0  |
| Sodium bisulfite                | 1.0   |
| Hydroquinone                    | 3.0   |
| Sodium carbonate (monohydrated) | 6.0   |
| Potassium bromide               | 0.80  |
| Water to make 1.0 liter.        |       |

In Table I are compared various development times 15 of the coatings containing the tetrahydropyran thioether of 2-mercaptopbenzothiazole on the one hand versus a typical antifogging agent on the other, that is, 2-phenylmercaptopbenzothiazole.

other 1½ hours. The reaction mixture was cooled and washed with sodium bicarbonate solution and with water. The solution was dried with  $\text{Na}_2\text{SO}_4$ , filtered and evaporated. The resulting syrup crystallized upon scratching with acetone. The crystals were recrystallized from n-propanol. Yield 14 g. yellow crystals=52%. Calc.  $\text{C}_{12}\text{H}_{13}\text{NS}_2\text{O}$ :

|   | Calc., percent | Found, percent |
|---|----------------|----------------|
| C | 58.67          | 57.2           |
| H | 5.23           | 5.7            |
| N | 5.7            | 5.7            |
| S | 26.1           | 27.7           |

Similarly treated was 5-mercaptop 2-phenyltetrazole (60 g.=1/3 mole). The yield was 57 g.=65%. Recryst. from MeOH. M.P. 101–103° C. Calc.  $\text{C}_{12}\text{H}_{14}\text{N}_4\text{SO}$ , M.W. 262.32.

TABLE I

| Coating number of test | Addenda                         | All tests developed in the developer of Example I |                        |                       |                        |                        |                        |                                              |                        |                                               |                        |
|------------------------|---------------------------------|---------------------------------------------------|------------------------|-----------------------|------------------------|------------------------|------------------------|----------------------------------------------|------------------------|-----------------------------------------------|------------------------|
|                        |                                 | Fresh tests                                       |                        |                       |                        |                        |                        | Aging tests                                  |                        |                                               |                        |
|                        |                                 | 3 minutes development                             |                        | 6 minutes development |                        | 12 minutes development |                        | Tank oven <sup>1</sup> 6 minutes development |                        | Pouch oven <sup>2</sup> 6 minutes development |                        |
|                        |                                 | Fog                                               | Speed at 0.2 above fog | Fog                   | Speed at 0.2 above fog | Fog                    | Speed at 0.2 above fog | Fog                                          | Speed at 0.2 above fog | Fog                                           | Speed at 0.2 above fog |
| 1                      | None                            | 0.13                                              | 65                     | 0.21                  | 91                     | 0.45                   | 91                     | 0.26                                         | 39                     | 0.14                                          | 73                     |
| 2                      | 1.63 mg. of TPT per mole Ag Br. | 0.9                                               | 70                     | 0.15                  | 91                     | 0.35                   | 117                    |                                              |                        |                                               |                        |
| 3                      | 3.25 mg. of TPT per mole Ag Br. | 0.9                                               | 64                     | 0.13                  | 110                    | 0.30                   | 129                    |                                              |                        |                                               |                        |
| 4                      | 6.5 mg. of TPT per mole Ag Br.  | 0.9                                               | 58                     | 0.11                  | 89                     | 0.26                   | 148                    |                                              |                        |                                               |                        |
| 5                      | 13.0 mg. of TPT per mole Ag Br. | 0.9                                               | 48                     | 0.9                   | 78                     | 0.16                   | 118                    |                                              |                        |                                               |                        |
| 6                      | 8.25 mg. of PMT per mole Ag Br. | 0.8                                               | 23                     | 0.8                   | 46                     | 0.10                   | 83                     |                                              |                        |                                               |                        |
| 7                      | 6.5 mg. of PMT per mole Ag Br.  | 0.6                                               | 12                     | 0.8                   | 26                     | 0.9                    | 46                     |                                              |                        |                                               |                        |
| 8                      | 6.5 mg. of TPT per mole Ag Br.  |                                                   |                        | 0.12                  | 88                     |                        |                        | 0.10                                         | 42                     | 0.14                                          | 126                    |
| 9                      | 6.5 mg. of PMT per mole Ag Br.  |                                                   |                        | 0.9                   | 29                     |                        |                        | 0.07                                         | 5                      | 0.19                                          | 40                     |

<sup>1</sup> Tank oven aging: The film was exposed to 75% relative humidity at 35° C. for 4 days.

<sup>2</sup> Pouch oven aging: The film was sealed into a plastic envelope at a relative humidity of 53% and kept at 49° C. for 6 days.

NOTE.—TPT equals tetrahydropyran ether of 2-mercaptopbenzothiazole; PMT equals phenylmercaptoptetrazole.

As can readily be ascertained, the tetrahydropyranether while functioning as an efficient antifogging agent does not suppress or cut down on the speed, whereas the phenylmercaptopbenzothiazole, although capable of retarding fog, also cuts prohibitively into the sensitivity and speed. From the incubation information, i.e., tank oven and pouch oven tests, it is at once evident that the tetrahydropyranethers are excellent stabilizing agents for retarding the degradation of photographic emulsions under conditions of excess humidity and temperature. Very little stabilizing effect is exhibited by the 2-phenylmercaptopbenzothiazole which, as previously pointed out, is a typical antifogging agent proposed by the prior art.

#### EXAMPLE II

The procedure of Example I was repeated with the exception that the tetrahydropyran thioether of Example I was replaced by the corresponding derivative of phenylmercaptoptetrazole. Results closely paralleled those of the earlier example.

#### Preparation of Tetrahydropyranthioethers

2-mercaptopbenzothiazole (16.3 g., 0.1 M) benzene (230 ml.) and p-toluene sulfonic acid 1/2 hydrate (0.15 g.) were refluxed for 30 minutes in a 1 liter 3-neck flask, equipped with stirrers, dropping funnel and a Dean and Stark trap. Refluxing was interrupted and dihydropyran (12 ml., 0.1 M) was added slowly (during 1 minute) through the dropping funnel. Refluxing was continued for an-

|   | Calc., percent | Found, percent |
|---|----------------|----------------|
| C | 54.94          | 55.34          |
| H | 5.38           | 5.56           |
| N | 21.36          | 21.31          |
| S | 12.22          | 12.04          |

55 I have also ascertained that the thioethers produced from 2,3-dihydrofuran are likewise effective as antifogging agents and/or stabilizers and in this respect resemble the previously described thioethers derived from dihydropyran. The synthesis of 2,3-dihydropyran in excellent yields is described in the chemical literature and in this connection reference is made to *Angewandte Chemie*, November 21, 1960, page 864. In forming the thioethers from 2,3-dihydrofuran the same procedure is employed as utilized in the preparation of the corresponding derivatives of the dihydropyran.

60 I claim:

65 1. A light sensitive photographic element comprising a base having thereon a light sensitive silver halide emulsion layer said element containing as an antifogging agent a compound of the following formula:



wherein R is selected from the class consisting of an alkyl group of from 1 to 20 carbon atoms, a benzyl group, a phenethyl group, a naphthylmethyl group, a cyclopentyl group, a cyclohexyl group, an aryl group selected from the class consisting of mono and bicyclic aromatic hydrocarbon radicals, a heterocyclic nucleus of the thiazole series, benzoxazole series, benzoselenazole series, quinoline series, benzimidazole series, tetrazole series and pyridine series and R<sub>1</sub> and R<sub>2</sub> are selected from the class consisting of hydrogen and an alkyl group from 1 to 20 carbon atoms.

2. The article as defined in claim 1 wherein said tetrahydropyran thioether is located in the silver halide emulsion.

3. The article as defined in claim 1 wherein said tetrahydropyran thioether is located in a layer adjacent to said silver halide emulsion.

4. A light sensitive photographic element comprising a base having thereon a light sensitive silver halide emulsion layer, said element containing as an antifogant and stabilizer a compound of the following formula:



25

5. The process of minimizing and preventing fog in a light sensitive silver halide material comprising a base having a light sensitive silver halide emulsion thereon which comprises exposing said emulsion to light and

30

20 2,855,301 Larson et al. Oct. 7, 1958

developing the same in the presence of an antifogant compound of the following formula:

5



wherein R is selected from the class consisting of an alkyl group of from 1 to 20 carbon atoms, a benzyl group, a phenethyl group, a naphthylmethyl group, a cyclopentyl group, a cyclohexyl group, an aryl group selected from the class consisting of mono and bicyclic aromatic hydrocarbon radicals, a heterocyclic nucleus of the thiazole series, benzoxazole series, benzoselenazole series, quinoline series, benzimidazole series, tetrazole series, and pyridine series and R<sub>1</sub> and R<sub>2</sub> are selected from the class consisting of hydrogen and an alkyl group of from 1 to 20 carbon atoms.

6. The process as defined in claim 5 wherein the antifogant and stabilizer is represented by the following formula:



25

References Cited in the file of this patent

UNITED STATES PATENTS

2,855,301 Larson et al. Oct. 7, 1958